

1

3,177,146

### FIRE-RESISTANT HYDRAULIC FLUIDS

Charles E. Francis, Martinez, Calif., assignor to Shell Oil Company, New York, N.Y., a corporation of Delaware  
No Drawing. Filed Oct. 17, 1961, Ser. No. 145,754  
10 Claims. (Cl. 252—75)

This invention relates to improved fire-resistant hydraulic fluids. More particularly, it pertains to water-in-oil colliery hydraulic fluids and lubricants which are fire and wear-resistant, stable and non-corrosive and to oil concentrates which are readily emulsifiable with large amounts of water.

Although it is known in the art that certain emulsions are useful as coolants and lubricants in metal working operations, the use of emulsion in hydraulic systems has been limited because of their inability to resist wear, their poor stability and their inability to pass fire-resistant requirements for which such fluids are primarily used.

In colliery equipment such as various hydraulic machinery, e.g., winder brake mechanism and wagon tipper to hydraulic jacks, pit props and roof bar straighteners, mechanical loaders and various other fluid drive mechanisms which are subject to load, shock and vibration, it is essential that the hydraulic fluid employed therein function properly and efficiently without the danger of being flammable or toxic.

A variety of so-called fire-resistant fluids are commercially available such as phosphate ester base fluids, but these have been found to possess poor low temperature viscosity-temperature properties, and they are toxic. Water-glycol solution or various water-oil emulsions have been found to have a tendency to form deposits and cause wear under high pressures and are costly. Also most emulsifiable oil concentrates when emulsified with hard water tend to form deposits which adversely affects the equipment.

It is an object of this invention to provide a composition which can be emulsified readily on the job to yield a fire resistant hydraulic fluid having good lubricating properties. Another object is to provide a fluid which after emulsification is a satisfactory lubricant for colliery hydraulic equipment, which is stable, non-toxic, fire-resistant, resistant to deterioration, inhibits corrosion and not cause wear. Still another object of this invention is to provide a water-mineral oil emulsion usable as lubricants and fire resistant hydraulic fluids for various equipment used in colliery hydraulic equipment. Still another object of this invention is to provide an oil concentrate which is readily emulsifiable with soft or hard water and capable of forming water-in-oil emulsions which are stable over a wide temperature range.

These and other objects are accomplished in accordance with this invention by providing a water-in-oil emulsion which comprises from about 20% to about 45% of water phase and from about 55% to about 80% of oil phase, the emulsion containing three essential additives namely two particular types of dissimilar non-ionic surface active agents and a water-soluble polymeric derivative of an acrylic acid represented by the formula:



where R is hydrogen or a  $\text{C}_{1-4}$  alkyl radical, R' and R'' may be hydrogen or lower alkyl radicals of up to 8 carbon atoms or they may be mixtures of hydrogen and a lower alkyl radical, M is a cation such as an alkali metal such as lithium, sodium or potassium, or ammonia or an organic base, x is a positive integer, y may be zero

2

or a positive integer and z may be zero or a positive integer, the molecular weight of the polymer varying from at least 1000 up to 500,000, preferably between 25,000 and 300,000. Instead of a polymer as represented by (I) a mixture of water-soluble homopolymers containing the desired groups



and



or polymers of (II) or (III) admixed with polyacrylic acid (IV).

The two non-ionic surface agents which are added to the mineral oil are (1) a monoester of a long chain fatty acid having at least 8 carbon atoms and an inner ether of aliphatic polyhydric alcohols such as hexahydric alcohols and (2) a polyalkyleneoxy phenoxy alkanol. Each of these additives must be present in critical amounts of which the monoester (1) is used in amounts ranging from 1% to 4%, preferably from 1.5% to 3% and the polyalkyleneoxy phenoxy alkanol (2) is used in amounts ranging from 0.5% to 3%, preferably from 1% to 2%.

In the monoester non-ionic surface agent the inner ether alcohol is prepared by partially dehydrating polyhydric alcohols which results in the conversion of the polyhydric alcohol to inner ether polyhydric compounds having 1 or 2 ethers and 4 to 6 hydroxyl groups in the molecule in the manner described in U.S. Patent 2,322,820. Compounds of this type are exemplified by sorbitan, mannitan, xylitan, dulcitan, etc. Fatty acids which are used to form the monoesters of the inner ether polyalcohols are saturated and unsaturated fatty acids having at least 8 carbon atoms, preferably from 12 to 18 carbon atoms, such as lauric, stearic, oleic, linoleic, ricinoleic acids and the like. Monoesters of this type include sorbitan monolaurate, sorbitan monostearate, sorbitan monooleate, sorbitan monoricinoleate, mannitan monolaurate, mannitan monooleate, and mixtures thereof. Compounds of this type are available commercially as "Span 20, 60 or 80" from the Atlas Powder Company.

The second essential additive is an oil-soluble alkyl phenoxy polyalkylene glycol having the formula



wherein n is an integer of from 2 to 6, preferably 3 to 4, R is an alkyl radical of 4 to 20 carbon atoms, preferably 4 to 12, and R' and R'' are the same or different alkylene groups such as ethylene or propylene groups, they are preferably the same, and preferably ethylene. Compounds of this type are  $\text{C}_{4-12}$  alkyl phenoxy(alkoxy)<sub>4-6</sub> alkanols exemplified by isobutylphenoxy tetraethylenoxy ethanol, diisobutylphenoxy tetraethylenoxy ethanol, nonylphenoxy tetraethylenoxy ethanol, octylphenoxy hexaethylenoxy ethanol, diisobutylphenoxy tripropyleneoxy propanol, and mixtures thereof.

The water-soluble copolymer or mixtures of homopolymer as defined by the above formulas can be prepared by any suitable means well known to the art. Thus the copolymers of Formula I can be prepared by copolymerizing a mixture of acrylic acid and acrylamide and reacting the copolymer with an alkali metal hydroxide to convert wholly or in part the acid groups to alkali metal carboxylate groups or an acrylamide may be polymerized and hy-

drolyzed in the presence of a polymerization catalyst and alkali metal hydroxide. The catalysts include inorganic or organic peroxides, or per-acids or azo catalysts such as hydrogen peroxide, diethyl peroxide, benzoyl peroxide, sodium or potassium persulfate, azo catalyst, e.g., alpha-alpha'-azodiisobutyronitrile, etc. and the alkali metal hydroxide includes sodium, potassium and lithium hydroxides. Thus a sodium polycarboxylate polyacrylamide (X) was prepared by admixing solutions of (a) aqueous solutions containing about 5500 parts of acrylamide and 4000 parts of water and (b) aqueous mixture of about 400 parts of sodium hydroxide, 70 parts of potassium persulfate and 900 parts water and reacting the two (a) and (b) at about 80° C. in the presence of an inert atmosphere. The product contained a mixture of acrylamide and sodium carboxyl groups and had a viscosity of 12,000-21,000 cps. Other water-soluble polymers in the molecular weight range of 5000-400,000 include sodium polyacrylate, sodium polymethacrylate, sodium polyacrylate-polyacrylic acid, potassium polyacrylate-polyacrylamide, potassium polymethacrylate-polymethacrylamide, sodium polyacrylate-N,N'-dimethylacrylamide, mixture of homopolymer of sodium polyacrylate and homopolymer of polyacrylamide (50/50), mixture of homopolymer of sodium polyacrylate and homopolymer of acrylic acid (60/40), mixture of polymer (X) and polyacrylic acid (Y) and the like.

Although water-soluble polymers of the above type are useful as thickeners, as polyelectrolytes, as flocculants, etc., their use in hydraulic systems with which the present invention is concerned is new, novel and unexpected. The polymers are dispersed in the water phase of emulsions of the present invention. They are added in amounts of from 0.01% to 2%, preferably from 0.05% to 1% of the water phase. In this manner emulsions are formulated by combining an oil concentrate with an aqueous solution or water containing the polymer to desired degree.

In addition to the above three essential additives it is preferred to use in such compositions small amounts of from about 0.01% to about 2%, preferably from about 0.2% to about 1% optional additives which include antioxidants and antiwear agents. The antioxidants include phenolic, amine and/or metal thiophosphate compounds. The phenolic compounds are illustrated by the alkyl phenols, e.g., di- and trialkyl phenols, for instance, 2,4-, 2,3-, 3,4-, and 2,6- and 3,5-diamylphenol, 2,4-dimethyl-6-tert. butylphenol, 2,6-ditert.butyl-4-methylphenol. The amines are illustrated in arylamines such as phenyl-alpha-naphthylamine or phenyl-beta-naphthylamine. The metal thiophosphates are illustrated by alkaline earth metal thiophosphates, e.g., calcium or zinc dimethyl cyclohexylidithiophosphate. The antiwear agents are sulfur-containing compounds such as oil-soluble polychloro hydrocarbyl thiocarbonate esters, e.g., polychloronaphtha methyl xanthate marketed by Monsanto Chemical Co. under the name "Santopoid S" and characterized by sp. gr. 1.19 at 60°/60° F., flash point 250° F., viscosity 63 cs. at 100° F., sulfur 11%, chlorine 31%. Thiocarbonates of this type are prepared by reacting a chlorinated petroleum naphtha with an alkali metal (potassium) amyl dithiocarbonate; organic sulfides such as dibenzyl disulfide or dichlorodibenzyl disulfide. Dyes and antifoaming agent can be added to composition of this invention. Oil-soluble dyes include naphthol yellow, Sandoz yellow, methylene blue, alizarin compounds, etc., while anti-foaming agents include silicone polymer (DC-200 fluids ranging in viscosity in centistokes from 100 to 1000 at 250° C.) or silicone type A fluid made by Dow-Corning Co. and described in U.S. Patents 2,563,588 and 2,662,055 and mixtures thereof.

The oil may be entirely a hydrocarbon oil of wide viscosity range, e.g., from less than 50 SUS at 100° F. to 150 SUS at 210° F. Oils of this type can be obtained from various crudes such as paraffinic, naphthenic or mixed base crudes; refined oils in the lubricating oil viscosity range are preferred. On the other hand, the hydrocarbon

oil may be blended with fixed oils such as castor oil, lard oil and the like and/or with synthetic lubricants such as polymerized olefins, organic esters of organic and inorganic acids, e.g., di-2-ethylhexyl sebacate, dioctyl phthalate, trioctyl phosphate; polymeric tetrahydrofuran, polyalkyl silicone polymer, e.g., dimethyl silicone polymer and the like. Where mixtures or blends are used the hydrocarbon oil such as a mineral lubricating oil is always present in the predominant amount such as from 60% to about 95% of the oil blend.

A straight mineral lubricating oil, having a viscosity index of at least 50 and ranging in viscosity at 100° F. of from 75 to 400 SUS, usually preferred. When it is derived from a lubricating oil stock of low viscosity index it is readily provided as raffinate in a selective solvent extraction process as is well understood in the art. The emulsion can be prepared by adding the required amount of water containing the polymeric compound as described to an oil containing the other two essential additives, while constantly stirring the mixture. Heating the emulsion during or after it is prepared is not necessary. If desired, the emulsion can be put through a homogenizer to insure a more stable emulsion. Instead of making the finished emulsion, the oil concentrate composition can be prepared and the required amount of water containing a polymeric compound as described added when the emulsion lubricant is ready for use. In this way storage and shipping costs can be reduced.

Illustrative examples of mineral oil bases of this invention which are emulsified with from about 20% to about 45%, preferably from about 30% to about 40% of water containing polymeric acylo compound to form a stable fire-resistant hydraulic fluid are presented below.

|                                                | Percent wt. |
|------------------------------------------------|-------------|
| Sorbitan monooleate                            | 2           |
| Diisobutylphenoxy(ethoxy) <sub>4</sub> ethanol | 1           |
| Mineral oil                                    | Balance     |
| Composition B:                                 |             |
| Sorbitan monostearate                          | 2           |
| Diisobutylphenoxy(ethoxy) <sub>4</sub> ethanol | 1           |
| Mineral oil                                    | Balance     |
| Composition C:                                 |             |
| Mannitan monooleate                            | 3           |
| Diisobutylphenoxy(ethoxy) <sub>4</sub> ethanol | 1           |
| Mineral oil                                    | Balance     |
| Composition D:                                 |             |
| Sorbitan monooleate                            | 2           |
| Diisobutylphenoxy(ethoxy) <sub>4</sub> ethanol | 1           |
| 2,6-ditert.butyl-4-methylphenol                | 0.2         |
| Phenyl-alpha-naphthylamine                     | 0.1         |
| Mineral oil                                    | Balance     |
| Composition E:                                 |             |
| Sorbitan monooleate                            | 2           |
| Diisobutylphenoxy(ethoxy) <sub>4</sub> ethanol | 1           |
| 2,6-ditert.butyl-4-methylphenol                | 0.2         |
| Phenyl-alpha-naphthylamine                     | 0.1         |
| Mineral oil                                    | Balance     |
| Composition F:                                 |             |
| Sorbitan monooleate                            | 2           |
| Diisobutylphenoxy(ethoxy) <sub>4</sub> ethanol | 1           |
| 4,4'-methylene(2,6-ditert.butylphenol)         | 0.2         |
| Phenyl-alpha-naphthylamine                     | 0.1         |
| Mineral oil                                    | Balance     |
| Composition G:                                 |             |
| Sorbitan monooleate                            | 3           |
| Diisobutylphenoxy(ethoxy) <sub>4</sub> ethanol | 1           |
| 4,4'-methylene(2,6-ditert.butylphenol)         | 0.2         |
| Phenyl-alpha-naphthylamine                     | 0.1         |
| Mineral oil                                    | Balance     |
| Composition H:                                 |             |
| Sorbitan monostearate                          | 1.5         |
| Diisobutylphenoxy(ethoxy) <sub>4</sub> ethanol | 1           |
| 4,4'-methylene(2,6-ditert.butylphenol)         | 0.2         |
| Phenyl-alpha-naphthylamine                     | 0.1         |
| Mineral oil                                    | Balance     |

The finished emulsion fluid is prepared by slowly adding to the oil base compositions such as A, B, C, D, E, F, G or H, from 20% to 45% based on the total composition, an aqueous base, such as water which contains 0.1% sodium polyacrylate-polyacrylamide (X) for compositions A, B and F, 0.05% sodium polyacrylate-polyacrylamide (X) for composition D, 0.1% potassium polyacrylate-polyacrylamide (X) for composition C, 0.2% polyacrylic acid + 0.1% sodium polyacrylate-polyamide (X) for composition E, 0.2% ammonium polyacrylate-polyacrylamide (X) for composition G and 0.1% lithium polyacrylate-polyamide (X) for composition H. The water base may or may not contain 0.01-1% of a corrosion or wear inhibitor such as water-soluble inorganic nitrates, nitrates, chromates, phosphates or water soluble low molecular weight salts such as alkali metal or alkaline earth metal (Na, K, Ca, Ba) acetate or propionate. The water-in-oil emulsion can be mixed by any suitable means such as by air agitation, propeller agitation or by passing through a colloid mill until a homogeneous stable water-in-oil emulsion is formed. For economical reasons, the water is added to the oil in desired amounts at the time the emulsion is to be used, although a stable water-in-oil emulsion can be prepared and stored for a moderate period.

A finished water-in-oil emulsion (Composition I) was prepared by admixing 60% of composition D with 40% water and the mixture was passed through a colloid mill until a stable homogeneous water-in-oil emulsion was formed.

Other finished compositions include:

| Composition II:                                      | Percent |
|------------------------------------------------------|---------|
| Water <sup>1</sup>                                   | 30      |
| Composition A                                        | 70      |
| Composition III:                                     |         |
| Water <sup>1</sup> containing 0.1% Ca acetate        | 40      |
| Composition G                                        | 60      |
| Composition IV:                                      |         |
| Water <sup>1</sup> containing 0.1% NaNO <sub>2</sub> | 35      |
| Composition C                                        | 65      |
| Composition V:                                       |         |
| Water <sup>1</sup>                                   | 40      |
| Composition E                                        | 60      |

<sup>1</sup> Water contains the corresponding water-soluble polymeric additive noted above used to blend with Compositions A to H, respectively and in amounts indicated.

Samples of Compositions I and V were stored in 100 ml. cylinders at 140° F. and observed for phase separation. The marked improvement in stability afforded by the inclusion of the polymers, as in Compositions I and V as compared to Composition W, is shown by Table I.

Table I

| Composition                   | I      |        | V   |        | W <sup>1</sup> |        |
|-------------------------------|--------|--------|-----|--------|----------------|--------|
|                               | Oil    | Water  | Oil | Water  | Oil            | Water  |
| Emulsion Stability at 140° F. |        |        |     |        |                |        |
| Separation, percent           |        |        |     |        |                |        |
| v.:                           |        |        |     |        |                |        |
| 1 day                         | slight | slight | 1   | slight | 1              | slight |
| 10 days                       | 1      | 1      | 5   | <1     | 15             | slight |
| 20 days                       | 3      | <1     | 9   | <1     | 37             | slight |
| 25 days                       | 3      | 2      | 11  | <1     | 45             | 2      |
| 30 days                       | 7      | 2      | 15  | <1     | -----          | -----  |
| 40 days                       | 9      | 2      | 18  | <1     | -----          | -----  |

<sup>1</sup> Composition W: [water-in-oil emulsion comprising 40% plus 60% mineral oil composition containing 2% sorbitan monooleate plus 1% diisobutylphenoxy (ethoxy)<sub>4</sub> ethanol plus 0.2% 2,6-di-tertiary-4-methyl phenol plus 0.1% phenyl alpha naphthylamine.]

Compositions of the present invention such as Compositions I through V are fire-resistant passing over 50 cycles as determined by the Pipe Cleaner Test described in Lubricating Engineering, March-April 1955, pages 86-87 while a neat mineral oil or a mineral oil containing 4% each of

Ca petroleum sulfonate and/or Ca C<sub>12-22</sub> alkyl salicylate ignited after 5 cycles.

I claim as my invention:

1. A water-in-oil emulsion lubricant and hydraulic fluid which is from about 20% to about 45% water phase consisting essentially of water and from about 0.01% to about 2% of a water-soluble polymeric compound having a molecular weight in the range from 1,000 to 500,000 and having the formula



where R is a radical selected from the group consisting of hydrogen and a C<sub>1-4</sub> alkyl radical, R' and R'' are radicals selected from the group consisting of hydrogen and an alkyl radical of up to 8 carbon atoms, M is a cation selected from the group consisting of an alkali metal, ammonium, and an organic base, x is a positive integer and y and z may be zero and positive integers, and from about 55% to about 80% oil phase, the oil phase being essentially a high viscosity index mineral oil having a viscosity in the range from 50 SUS at 100° F. to 150 SUS at 210° F. containing (1) from about 1% to about 4% of a monoester of a long chain fatty acid having at least 8 carbon atoms and an inner ether of an aliphatic polyhydric alcohol having 1-2 ether and 4-6 hydroxyl groups, and (2) from about 0.5% to about 3% of an oil-soluble alkyl phenoxy polyalkylene glycol having the formula R-phenyl(-OR')<sub>n</sub>-OR''-OH where R is an alkyl radical having 4 to 20 carbon atoms; and R' and R'' are alkylene groups having 2 to 3 carbon atoms; and n is an integer of from 2 to 6.

2. A water-in-oil emulsion lubricant and hydraulic fluid which is from about 20% to about 45% water phase consisting essentially of water and from about 0.01% to about 2% of a water-soluble alkali metal polyacrylate having a molecular weight in the range from 25,000 to 300,000, and from about 55% to about 80% oil phase, the oil phase being essentially a 80-100 V.I. mineral oil having a viscosity in the range from 75 to 400 SUS at 100° F. containing (1) from about 1.5% to about 3% of a monoester of a fatty acid from 12 to 18 carbon atoms and an inner ether of an aliphatic hexahydric alcohol having 1-2 ether and 4-6 hydroxyl groups and (2) from about 1% to about 2% of an oil-soluble C<sub>4-12</sub> alkyl phenoxy(ethoxy)<sub>4-6</sub>ethanol.

3. The composition of claim 2 containing in the emulsion from 0.01% to 2% of an oil-soluble antioxidant selected from the group consisting of alkyl phenols, phenyl-alpha-naphthylamine, and mixtures thereof, said alkyl phenols having 2 to 3 alkyl groups having from 1 to 5 carbon atoms.

4. A water-in-oil emulsion lubricant and hydraulic fluid which is from about 20% to about 45% water phase consisting essentially of water and from about 0.01% to about 2% of a water-soluble alkali metal polyacrylate-polyacrylamide having a molecular weight in the range from 25,000 to 300,000, and from about 55% to about 80% oil phase, the oil phase being essentially a 80-100 V.I. mineral oil having a viscosity in the range from 75 to 400 SUS at 100° F. containing (1) from about 1.5% to about 3% of a monoester of a fatty acid having from 12 to 18 carbon atoms and an inner ether of an aliphatic hexahydric alcohol having 1-2 ether and 4-6 hydroxyl groups and (2) from about 1% to about 2% of an oil-soluble C<sub>4-12</sub> alkyl phenoxy(ethoxy)<sub>4-6</sub>ethanol.

5. The composition of claim 4 containing in the emulsion from 0.01% to 2% of an oil-soluble antioxidant selected from the group consisting of alkyl phenols, phenyl-alpha-naphthylamine, and mixtures thereof, said alkyl phenols having 2 to 3 alkyl groups having from 1 to 5 carbon atoms.

6. A water-in-oil emulsion lubricant and hydraulic fluid which is from about 20% to about 45% water phase consisting essentially of water and from about 0.01% to about 2% of a water-soluble alkali metal polyacrylate-polyacrylic acid having a molecular weight in the range from 25,000 to 300,000, and from about 55% to about 80% oil phase, the oil phase being essentially a 80-100 V.I. mineral oil having a viscosity in the range from 75 to 400 SUS at 100° F. containing (1) from about 1.5% to about 3% of a monoester of a fatty acid having from 12 to 18 carbon atoms and an inner ether of an aliphatic hexahydric alcohol having 1-2 ether and 4-6 hydroxyl groups and (2) from about 1% to about 2% of an oil-soluble C<sub>4-12</sub> alkyl phenoxy(ethoxy)<sub>4-6</sub>ethanol.

7. A water-in-oil emulsion lubricant and hydraulic fluid which is from about 20% to about 45% water phase consisting essentially of water and from about 0.02% to about 1% of a water-soluble sodium polyacrylate-polyacrylamide having a molecular weight in the range from 25,000 to 300,000, and from about 55% to about 80% oil phase, the oil phase being essentially a 80-100 V.I. mineral lubricating oil having a viscosity in the range from 75 to 400 SUS at 100° F. containing from about 1.5% to about 3% of a sorbitan monooleate and from about 1% to about 2% of C<sub>4-12</sub> alkyl substituted mixture of phenoxy(ethoxy)<sub>4-6</sub>ethanol.

8. A water-in-oil emulsion lubricant and hydraulic fluid which is from about 20% to about 45% water phase consisting essentially of water and from about 0.02% to about 1% of a water-soluble sodium polyacrylate-polyacrylic acid having a molecular weight in the range from 25,000 to 300,000, and from about 55% to about 80% oil phase, the oil phase being essentially a

80-100 V.I. mineral lubricating oil having a viscosity in the range from 75 to 400 SUS at 100° F. containing from about 1.5% to about 3% of a sorbitan monooleate, and from about 1% to about 2% of a C<sub>4-12</sub> alkyl substituted mixture of phenoxy(ethoxy)<sub>4-6</sub>ethanol.

5 9. The composition of claim 8 containing in the emulsion from about 0.01% to about 1% each of 2,6-ditert.butyl-4-methylphenol, phenyl-alpha-naphthylamine and zinc diamyldithiocarbamate.

10 10. A water-in-oil emulsion lubricant and hydraulic fluid which is from about 30% to about 40% water phase consisting essentially of water and from about 0.02% to about 1% of a water-soluble sodium polyacrylate-polyacrylamide having a molecular weight in the range from 25,000 to 300,000, and from about 70% to about 60% oil phase, the oil phase being essentially a 80-100 V.I. mineral lubricating oil having a viscosity in the range from 75 to 400 SUS at 100° F. containing from about 1.5% to about 3% of sorbitan monooleate, and from about 1% to about 2% of an oil-soluble diisobutylphenoxy(ethoxy)<sub>4-6</sub>ethanol.

#### References Cited by the Examiner

##### UNITED STATES PATENTS

|              |                    |          |
|--------------|--------------------|----------|
| 25 2,868,728 | 1/59 Hotten et al. | 252-33.6 |
| 30 3,050,465 | 8/62 Francis       | 252-49.5 |

##### FOREIGN PATENTS

|         |                     |
|---------|---------------------|
| 801,411 | 9/58 Great Britain. |
|---------|---------------------|

30 ALBERT T. MEYERS, *Primary Examiner.*

JOSEPH H. LIBERMAN, JULIUS GREENWALD,  
Examiners.